

April 4, 1950

A. F. PRUST

2,503,217

PROCESS FOR TREATING BRIGHTENED ELECTROTINPLATE

Filed Dec. 15, 1944



INVENTOR.  
ALVIN FREDERICK PRUST

BY

*Rickey Watts*  
ATTORNEYS

## UNITED STATES PATENT OFFICE

2,503,217

## PROCESS FOR TREATING BRIGHTENED ELECTROTINPLATE

Alvin Frederick Prust, Warren, Ohio, assignor to Republic Steel Corporation, Cleveland, Ohio, a corporation of New Jersey

Application December 15, 1944, Serial No. 568,241

5 Claims. (Cl. 204—141)

1

This invention relates generally to the tinplate art and particularly to a new and improved method of and apparatus for treating the surfaces of electro-tinplate.

Electro-tinplate, that is, steel having surface coatings of electro-deposited tin, as made herefore, does not adhere strongly or uniformly to enamel or lacquer. When such surfaces have been brightened, as by being fused after electro-deposition of the tin, they often become discolored with a yellow discoloration, and there is a tendency for lacquer or enamel which has been baked thereon to loosen from the tin or actually to flake off. I believe that when electro-tinplate is brightened the surface layers of the tin are activated and oxidized; and that when such a surface is enameled or lacquered, at temperatures which may range up to about 420° F., the oxide on or the oxidation of the tin surface layer forms a weak connection between the enamel or lacquer and the tin which is not strong enough to prevent the coating material from loosening or flaking off.

The present invention aims to avoid those causes of poor adherence and provides a method of and apparatus for treatment of brightened electro-tinplate so that enamel or lacquer will adhere tenaciously due, I believe, to the passive or non-oxidized condition of the surface layers of the tin.

Briefly stated, the present invention comprises a treatment of brightened electro-tinplate which converts the surface layer of the tin into a de-oxidized and passive state, that is, deoxidizes it and makes it resistant to oxidation, and protects it against oxidation as evidenced by discoloration, even when heated to a lacquering temperature of about 420° F. This method of treatment comprises the steps of making a brightened electro-tinplate article the cathode in a heated electrolyte containing hexavalent chromium and passing a low density current thru the electrolyte, surrounding the article with a non-oxidizing atmosphere while washing and largely drying it, flash heating it to complete drying and then coating it with a protective coating.

An illustrative, but not limiting, set of conditions under which the present invention has been satisfactorily practiced is as follows: A piece of electro-tinplate with brightened surfaces, the brightening having been accomplished by fusing the deposited tin, was made the cathode in an electrolytic bath, the anodes being composed of low carbon steel. The electrolyte consisted of water containing between about .5% and

2

about .75% by weight of potassium chromate. A current of between about 10 and about 15 amperes per sq. ft. and at a voltage of about 7.5 volts was passed thru the electrolyte and piece of tinplate for about one second. The strip was then washed, largely dried in a steam atmosphere, finally and rapidly dried, and immediately coated with oil. The electrotinplate so heated did not exhibit any tendency to develop a yellow coloration when heated at about 420° F. for about twenty minutes and enamel and lacquer baked on the thus treated tinplate adhered tenaciously and uniformly to the tinplate and exhibited no tendency to flake off.

15. It will be understood that the specific conditions set out in the foregoing example may be modified considerably and within the following limits:

The temperature of the electrolyte may range 20 between about 150° F. and about 200° F. Temperatures lower than about 150° F. may be used but are not desirable. In general, temperatures much below about 180° F. are not desired because the current requirements increase in inverse proportions to the decrease in temperature.

The length of time the current is flowing thru any part of the article may range from 25 about one-half second to about ten seconds. This range of time is apparently determined by the time required for the electrolyte to change sufficiently to attack the tin. It appears that the nature of the diffusion layer or cathode film is a function of the applied current density and time of treatment. With a constant current density, the pH value or alkalinity of the diffusion layer rises in proportion to the time of treatment until its alkalinity becomes high enough to attack the tin. With current densities 30 within the range later specified herein, a treatment time of as much as about ten seconds is not sufficiently long to cause any bad effects on the tinplate resulting from an attack of the tin by the electrolyte.

40. Current densities may be used which range from about 4 to about 25 amperes per sq. ft. with the best results being obtained within the range of from about 10 to 18 amperes per sq. ft.

45. Since the voltage is a function of the required current density and the concentration and temperature of the electrolyte, the ranges of voltages are fairly well defined by those factors. However, in general, it may be said that for the ranges of current density and concentration and 50 temperature of the solutions as set out herein

the ordinarily available voltages of from about .5 volt to about 18 volts are satisfactory.

In lieu of the potassium chromate mentioned in the foregoing illustration any other water soluble hexavalent compound of chromium may be used including sodium chromate, a dichromate of either sodium or potassium, or chromic acid. The concentration of the chromium ions in the electrolyte may range between those present in from about .5% to about 5% by weight of potassium chromate. However, it will be understood that these limits are not necessarily controlling because they will obviously vary depending on the voltage employed, the manner of rinsing the treated tinplate and the speed of travel of the tinplate thru the electrolyte. The limits just stated have been found to be satisfactory with tinplate traveling thru the electrolyte at the rate of about 100 to about 800 ft. per minute, with ordinary rinsing practice and with the voltages maintained within the foregoing limits.

The present process has been carried out successfully on a commercial scale under the following set of conditions: Electro-tinplate in endless strip form was passed at a speed of 250 ft. per minute, thru an electrolyte containing about .75% of potassium chromate by weight while a current of about 4.5 volts and an amperage of about 10 to 18 amperes per sq. ft. was flowing thru the electrolyte and tinplate. The temperature of the electrolyte was about 180° F. The strip moved from the electrolyte thru a steam atmosphere into and out of a body of wash water and between steam jets which removed practically all the wash water and electrolyte from its surfaces. Then it was heated for a fraction of a second and thereby made substantially dry and immediately thereafter it was coated with an oil emulsion and heated to dry out that coating.

The present invention will be better understood by those skilled in the art from the following description of the construction and operation of the apparatus illustrated in the drawing which is attached to and forms a part of this specification.

In the figure tinplate in the form of an elongated strip 1 passes from roll stand 2 between roll 3 and cathode roll 4 which constitutes part of an electric circuit. From roll 3 strip 1 moves vertically down between anodes 5, also in the electric circuit, and around roll 6 and thence upwardly to roll 7. The anodes 5 and roll 6 are positioned in a cell 8 which is substantially full of electrolyte. The strip 1 passes from roll 7 down to and around roll 9 and thence up to roll 10. Roll 9 is located near the bottom of cell 11 which is partly filled with condensed steam containing more or less electrolyte. The temperature of the electrolyte is controlled by heating coils 12 in the upper portion of cell 8 and the temperature of the liquid in cell 11 is controlled by heating coils 13 near the bottom of that cell. A hood 14 encloses the upper end of cell 11 and part of cell 8, and serves to retain a steam atmosphere around the strip in both cells above the surface of liquids therein. Just below roll 10 pipes 15 are disposed on opposite sides of the strip 1 and are provided with openings thru which steam may be discharged against the surfaces of the strip at an acute angle and in a direction opposite to the direction of travel of the strip as it moves from roll 9 to roll 10.

Immediately after leaving roll 10, strip 1 passes

between flash heater tubes 16 which extend along the strip for a distance of a little less than two feet. Then the strip passes into a spray chamber 17 where an oil emulsion is sprayed onto the surfaces of the strip thru perforations in tubes 18. Excess oil emulsion collects in tank 19 below this spray chamber 17 and may be repumped thru pipes 18. When the strip 1 leaves chamber 17 it passes under roll 20 which dips into water in rinse tank 21 therebeneath and then passes upwardly between inclined heating tubes 22.

It will be understood that the flow brightened, oxidized, tinplate surfaces are deoxidized in passing between anodes 5 in the electrolyte in cell 8; that the strip is then protected against contact with the air while passing from the electrolyte into and out of the liquid in cell 11; that the electrolyte is washed from the strip by the liquid in cell 11 and most of the moisture is removed from the strip by the jets of steam from steam pipes 15; that the remaining moisture on the strip is driven off by flash heating, that is, by being heated for not more than about one second by the heater pipes 16; that immediately thereafter the surfaces of the strip are coated with a water-oil emulsion and the emulsion is spread more or less uniformly over the surfaces by the water in the rinse tank, after which heaters 22 evaporate water from the emulsion and dry the oil of the emulsion which remains as an adherent coating on the strip.

As has been stated above, I believe that the foregoing treatment not only reduces any oxides which may be on the surface of the brightened electro-tinplate but also makes the surface layers of the tin passive or protects them to such an extent that they do not become oxidized to a material extent either before or during subjectation to the oven temperatures at which lacquer or enamel is baked thereon. I believe that it is due to this reduction and passivation of the surface layers of the tin and the protection afforded by the non-oxidizing atmosphere and the final coating that the strong, tenacious adherence of enamel and lacquer to tinplate treated by this method is largely, if not entirely, traceable.

This application is a continuation-in-part of my copending application Ser. No. 520,783 filed February 2, 1944, now abandoned.

Having thus described my invention so that others skilled in the art may be able to understand and practice the same, I state that what I desire to secure by Letters Patent is defined in what is claimed.

55. What is claimed is:

1. The method of treating elongated brightened electro-tinplate which comprises the steps of making the tinplate a cathode, moving such tinplate endwise and successively deoxidizing tin surfaces thereof electrolytically in an aqueous, hexavalent chromium electrolyte, covering the thus deoxidized surfaces with a steam atmosphere while passing the tinplate from the electrolyte into and out of a body of washing liquid and thereby protecting said surfaces by said atmosphere against oxidation and substantially completely drying them after they pass out of the washing liquid, heating said surfaces for less than about one second to remove final moisture therefrom and forming an oil coating on said surfaces.

2. The method of treating elongated brightened electro-tinplate which comprises the steps of making the tinplate a cathode, moving such tinplate endwise and successively deoxidizing tin surfaces thereof electrolytically in an aqueous,

hexavalent chromium electrolyte, covering the thus deoxidized surfaces with a steam atmosphere while passing the tinplate from the electrolyte into and out of a body of washing liquid and thereby protecting said surfaces by said atmosphere against oxidation and substantially completely drying them after they pass out of the washing liquid, heating said surfaces for less than about one second to remove final moisture therefrom, forming an oil coating on said surface, rinsing said coating in water and drying the coating.

3. The method of treating elongated brightened electro-tinplate which comprises the steps of making the tinplate a cathode, moving such tinplate endwise and successively deoxidizing tin surfaces thereof electrolytically in an aqueous, hexavalent chromium electrolyte, covering the thus deoxidized surfaces with a steam atmosphere while passing the tinplate from the electrolyte into and out of a body of washing liquid and thereby protecting said surfaces by said atmosphere against oxidation and substantially completely drying them after they pass out of the washing liquid, heating said surfaces for less than about one second to remove final moisture therefrom, forming an oil coating on said surfaces and drying the coating.

4. The method of treating brightened electro-tinplate which comprises the steps of removing oxides from surfaces of such tinplate by making the tinplate the cathode in an aqueous electrolyte containing dissolved hexavalent chromium ions equivalent to those in from .5% to .75% by weight of alkali chromate and passing an electric current of from about 4 amps. to about 25 amps. per sq. ft. thru said electrolyte and tinplate for between about one second and about ten seconds, removing electrolyte from the tin surfaces by passing the tinplate in a steam atmosphere into and out of a body of water, removing water from said surfaces by directing jets of steam under pressure at an acute angle thereagainst, drying the tin surfaces by heating them for less than one second and immediately protecting the tin surfaces against contact with air by covering them with an adherent oil emulsion film and removing moisture from said film.

5. The method of treating elongated brightened electro-tinplate, which comprises the steps of moving said tinplate endwise at a lineal speed

of from about 100 to about 800 feet per minute and successively treating increments thereof as follows: removing oxides from surfaces of such tinplate by making it the cathode in an aqueous electrolyte containing dissolved hexavalent chromium ions equivalent to those in from .5% to .75% by weight of alkali chromate and maintained at a temperature of between about 150° F. and about 200° F. and passing an electric current of from about 4 amps. to about 25 amps. per sq. ft. thru said electrolyte and tinplate for between about one second and about ten seconds, removing electrolyte from the tin surfaces by passing the tinplate in a steam atmosphere into and out of a body of water at a temperature of about 180° F., removing water from said tin surfaces by directing jets of steam under pressure at an acute angle thereagainst, drying the tin surfaces by heating them for less than one second, covering the tin surfaces with an oil emulsion film, rinsing in water and heating said film.

ALVIN FREDERICK PRUST.

#### REFERENCES CITED

25 The following references are of record in the file of this patent:

#### UNITED STATES PATENTS

| Number       | Name         | Date           |
|--------------|--------------|----------------|
| 30 1,827,204 | Mason        | Oct. 13, 1931  |
| 1,872,614    | Wirshing     | Aug. 16, 1932  |
| 2,125,387    | Mason        | Aug. 2, 1938   |
| 2,142,486    | Antisell     | Jan. 3, 1939   |
| 35 2,203,062 | Schueller    | June 4, 1940   |
| 2,215,143    | Clayton      | Sept. 17, 1940 |
| 2,215,165    | Sumner       | Sept. 17, 1940 |
| 2,234,593    | Ferm et al.  | Mar. 11, 1941  |
| 2,255,859    | Quigley      | Sept. 16, 1941 |
| 2,266,330    | Nachtman     | Dec. 16, 1941  |
| 30 2,274,963 | Hopper       | Mar. 3, 1942   |
| 2,306,143    | Stevenson    | Dec. 22, 1942  |
| 2,314,818    | Cook et al.  | Mar. 23, 1943  |
| 2,317,242    | Allen et al. | Apr. 20, 1943  |
| 2,327,127    | Rath         | Aug. 17, 1943  |
| 45 2,327,885 | Grace et al. | Aug. 24, 1943  |
| 2,424,718    | Stevenson    | July 29, 1947  |

#### FOREIGN PATENTS

| Number     | Country       | Date         |
|------------|---------------|--------------|
| 50 479,746 | Great Britain | Feb. 7, 1938 |